

# United States Patent

[11] 3,613,100

[72] Inventors **Helmut Kaufer**  
Metzkausen ueber Mettmann;  
Erich Berger, Unterhaching Munich; Hans-  
Peter Huber, Munich, all of Germany  
[21] Appl. No. **444,875**  
[22] Filed **Apr. 1, 1965**  
[45] Patented **Oct. 12, 1971**  
[73] Assignee **Agfa Aktiengesellschaft**  
Leverkusen, Germany  
[32] Priority **Apr. 4, 1964**  
[33] **Germany**  
[31] **A 45665 IXG/21 A**

[50] **Field of Search**..... 346/1, 74  
M, 74 MD; 179/100.2 A; 274/41.4; 117/235;  
101/DIG. 13, 310/4; 178/6.6 A; 340/174.1

[56] **References Cited**  
UNITED STATES PATENTS  
2,643,130 6/1953 Kornel..... 274/41.4  
2,793,135 5/1957 Sims et al..... 117/17.5  
3,176,278 3/1965 Mayer ..... 340/174.1  
3,364,496 1/1968 Greiner et al..... 346/74

*Primary Examiner*—Joseph W. Hartary  
*Attorney*—Michael S. Striker

[54] **METHOD AND DEVICE FOR MAGNETIC IMAGE FORMATION**  
29 Claims, 20 Drawing Figs.

[52] **U.S. Cl.**..... **346/1**,  
346/74, 117/235, 117/17.5, 101/426, 340/174.1  
[51] **Int. Cl.**..... **G11b 5/02**

**ABSTRACT:** Recording means for magnetic data recording which include at least two magnetic materials of different temperature dependency with respect to at least one magnetic characteristic of the same, and a method of operating a device of such type for storing magnetic recording which includes subjecting the recording means, particularly the two magnetic materials of different temperature dependency to the influence of a magnetizing or demagnetizing field.



PATENTED OCT 12 1971

3,613,100

SHEET 01 OF 11



INVENTORS

BY  
HELMUT KÄUFER  
ERICH BURGER  
HANS PETER HUBER

*Michael J. Strite  
N.Y.*

PATENTED OCT 12 1971

3,613,100

SHEET 02 OF 11



Fig. 2

**INVENTORS**

BY  
HELMUT KÄUFER  
ERICH BURGER  
HANS PETER HUBER

Michael J. Strick  
Att'n:

PATENTED OCT 12 1971

3,613,100

SHEET 03 OF 11



Fig. 3



Fig. 4



Fig. 5

INVENTORS

BY  
HELmut KÄUFER  
ERICH BURGER  
HANS PETER HUBER

*Michael J. Striker  
N.Y.*

PATENTED OCT 12 1971

3,613,100

SHEET 04 OF 11



Fig. 6



Fig. 7

INVENTORE  
HELmut KÄUFER  
ERICH BURGER  
HANS PETER HUBER

BY

Michael J. Striker  
P.M. 7

PATENTED OCT 12 1971

3,613,100

SHEET 05 OF 11

Fig.8



Fig.9



INVENTORE  
BY  
HELMUT KÄUFER  
ERICH BURGER  
HANS PETER HUBER

Michael J. Strick  
N.Y. 7

PATENTED OCT 12 1971

3,613,100

SHEET 06 OF 11



Fig.10

INVENTORE  
BY  
HELmut KÄUFER  
ERICH BURGER  
HANS PETER HUBER

Michael J. Strick  
N.M.

PATENTED OCT 12 1971

3,613,100

SHEET 07 OF 11

Fig.11



Fig.12



Fig.13

INVENTORS

BY  
HELmut KÄUFER  
ERICH BURGER  
HANS PETER HUBER

Michael J. Strite  
N.Y.,

PATENTED OCT 12 1971

3,613,100

SHEET 08 OF 11



INVENTORS  
BY  
HELMUT KAUFER  
ERICH BURGER  
HANS PETER HUBER

Michael J. Strickler  
N.Y.



INVENTORS  
BY  
HELMUT KÄUFER  
ERICH BURGER  
HANS PETER HUBER

*Michael J. Striker  
N.Y.*

PATENTED OCT 12 1971

3,613,100

SHEET 10 OF 11



Fig. 18



Fig. 20

INVENTORS  
HELMUT KÄUFER  
ERICH BURGER  
HANS PETER HUBER  
BY

Michael J. Stibor  
A.M.



BY

## INVENTORS

HELMUT KÄUFER  
 ERICH BURGER  
 HANS PETER HUBER

Michael J. Stricker  
 N.M.

**METHOD AND DEVICE FOR MAGNETIC IMAGE FORMATION**

The present invention relates to a method and device for magnetic image formation. More particularly, the present invention is concerned with a magnetic storage means or device for magnetic recording wherein the recording is produced with the help of the temperature dependency of a magnetic characteristic of a magnetic material contained in the storage device.

It has already been proposed to carry out magnetic data recording by heating selective portions of a conventionally premagnetized recording layer above their Curie point. It has also been proposed to form a magnetic image under utilization of the temperature dependency of the permeability of a magnetizable material.

It is an object of the present invention to provide a method and device for preparing latent magnetic images corresponding to an original image, and for forming from such latent magnetic image a reproduction of the original image, which device can be easily produced and which method can be carried out in a relatively simple manner, while lending itself to a great variety of practical usages, including, for instance, the forming of multicolor copies of multicolor original images, as well as for halftone copying of images comprising a variety of shades of gray.

Other objects of the present invention, as well as various further practical applications of the same will become apparent from a further reading of the description and of the appended claims.

With the above and other objects in view, the present invention broadly includes recording means for magnetic data recording, the recording means including at least two magnetic materials of different temperature dependency with respect to at least one magnetic characteristic of the same.

The present invention also contemplates in a device for storing magnetic recordings wherein the temperature dependency of a magnetic characteristic of a magnetic material is utilized for magnetic data recording, recording means for magnetic data recording including at least two magnetic materials of different temperature dependency of their magnetic permeability.

The present invention also provides in a method of preparing a latent image steps of forming a layer including portions of different magnetizable materials in the region of the face of the layer, the magnetic characteristics of each of the materials being adapted to be changed by heating the materials to at least a predetermined different temperature, respectively, and heating the face of the layer selectively to different ones of the predetermined different temperatures in such a manner that each of the different ones of the predetermined different temperatures corresponds to a selected characteristic of an image to be reproduced, so as to change the magnetic characteristics of the materials of those particles which are heated to at least their respective predetermined temperatures, whereby the distribution in the layer of different magnetizable materials the magnetic characteristics of which have been changed corresponds to the distribution of the selected characteristics of the image to be reproduced.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawings, in which:

FIGS. 1 and 2 are graphic illustrations of the temperature dependency of the permeability and of the coercive force of various materials, mixtures of which may be incorporated in the magnetic recording layer;

FIGS. 3-5 schematically illustrate the structure of mixed layers formed of hard magnetic constituents and of soft magnetic constituents, the permeability of the latter being temperature dependent;

FIG. 6 is a schematic illustration of the manner in which a latent magnetic image corresponding to a colored original image appears in a magnetic recording layer according to the present invention;

5 FIG. 7 is a graphic representation of the temperature dependency of the individual components of the layer of FIG. 6;

FIG. 8 is a schematic illustration of the forming of a colored image on a recording layer carrying or holding a corresponding latent magnetic image;

10 FIG. 9 illustrates the selective application of various colors after stepwise heating of the carrier of the latent magnetic color image;

FIGS. 10-12 serve to schematically illustrate the structure and manner of operation of inking arrangements which respond to selected magnetic field strengths;

15 FIG. 13 is a schematic illustration of a segment of a magnetically produced halftone block;

FIGS. 14-17 are schematic and graphic representations of the manner in which the latent magnetic image may be produced under utilization of external magnetic fields of different strength;

20 FIG. 18 is a schematic illustration of a magnetic recording layer according to the present invention wherein each of the particles of magnetic material comprises a core with two superposed cover layers around the same;

25 FIG. 19 is a graphic illustration of the correlation between the color separations of an original colored image and the temperature stages of a layer containing magnetic particles comprising a core portion and a covering layer; and

30 FIG. 20 is a schematic illustration of an arrangement for multiple form printing with changes in the printed matter of different forms of each set.

According to the present invention it is proposed to form a 35 magnetic recording layer which contains at least two different magnetic materials which differ with respect to the temperature dependency of their magnetic properties. Thereby a storage device for magnetic recordings is provided which may be used in many different ways and achieve a variety of results 40 which cannot be achieved with a recording layer containing only a single magnetic material.

The storage means or device for magnetic recordings will contain, in accordance with the present invention, for instance, at least one soft magnetic material the permeability of 45 which is temperature dependent within the operating temperature of the recording means, and at least one hard magnetic material which has a Curie point above the range of operating temperatures of the storage means for magnetic recordings.

50 It is possible to produce in such layer by very small temperature differentials very great differences in the permanent magnetization of the individual portions of the layer when the layer is subjected to a uniform external magnetic field. The permeable portions of the layer, the permeability of which may change within a few degrees Centigrade by three powers of 10 are capable of nearly completely shielding the hard magnetic constituents of the layer against the effect of external magnetizing or demagnetizing fields, at such portions of the 55 layer where permeable constituents are interposed between the source of the magnetic field and the hard magnetic constituents, or where the hard magnetic constituents are covered by permeable constituents. In addition, by means of this blocking or bypass effect disturbing effects of the reading 60 means or scanning arrangement on the recording are largely repressed. For instance, for effectively erasing a magnetic printing form, an opposing magnetic field of about twice the strength of the latent magnetic image would be required.

When, however, a permanently magnetic particle is blocked 65 with a factor of 100 by surrounding material of temperature dependent permeability, then the retroaction of an opposing magnetic field of double the strength of the field formed by the permanently magnetic or hard magnetic particle, will equal only one five-thousandth of the magnetization of the 70 particle carrying the magnetic recording.

This means that the normal effect of the magnetization of the hard magnetic portions of the recording layer will be reduced only by the blocking ratio, while the reactive disturbance of an external field is reduced by about the square of the blocking ratio. Thus, a true increase in the stability or resistance to unwanted erosion is obtained which may be utilized in connection with all magnetic storage means which cooperate with a reading or scanning device, for instance in computers, sound recording devices and the like. It is also possible to subject such a magnetic storage device also in stationary condition to scanning with a strong external alternating field, for instance a filed probe according to Brankoff. Such storage devices for magnetic recordings, when in cold condition are thus also effectively protected against unwanted external fields.

When a signal field is available for magnetizing the magnetic storage layer, which field is stronger than the blocking factor, heating during recording will not be necessary.

When, however, primarily the thermal control effect of the mixed magnetic layer and its increased resistance to magnetic fields is to be utilized, then, during recording, the layer may be heated corresponding to the image to be recorded, and during reading, the layer may be evenly heated, in both cases to a temperature above the Curie point of the soft magnetic constituents of the layer.

These soft magnetic constituents act then only as simple magnetic resistance and, due to their small cross-sectional dimension, will permit external and internal magnetic fields to exert a nearly full strength effect.

The present invention further proposes that the storage device for magnetic recordings includes at least one soft magnetic material the permeability of which is temperature dependent within the range of operating temperatures of the recording device, and at least one hard magnetic material having a Curie point within the range of operating temperatures of the device or method. In this case, the recording layer will have several operating temperatures of which, for instance, one may be utilized for controlling the magnetic recording, while another operating temperature may serve for complete or partial erasure of the recording. This system may be used, for instance, for multiple form printing with changes in the printed matter of different forms of each set.

According to a further embodiment of the present invention, the magnetic storage device or recording layer may contain at least two hard magnetic materials of different coercive force, or at least one of the soft magnetic materials may possess within the range of operating temperatures of the recording layer an essentially linear increase or decrease of its permeability. Such layers permit to correlate to each temperature range a certain recording magnetic field strength, and this may be utilized, for instance, for superposed copying of several halftone separations on one printing form or copy sheet. Similar effects can be achieved when the recording layer contains at least two hard magnetic materials of different Curie point and different coercive force, provided that the layers have been premagnetized.

According to a preferred embodiment of the present invention, the hard magnetic particles are embedded in a soft magnetic layer. This arrangement, whereby preferably the hard magnetic particles are completely surrounded by the soft magnetic material, will result in an excellent blocking effect. In this manner a spatial or three-dimensional lattice is formed having a total resistance which remains substantially the same for each direction of an external magnetic field, due to the parallel connection of the individual magnetic resistances and due to the bending of the lines of flux or magnetic force at the separating surfaces between the two constituents of different permeability. This is of significant importance, particularly in connection with the magnetizing arrangement which is frequently utilized for magnetic data storage, for instance for sound recording tape, wherein two magnetic poles are arranged at one and the same side of the layer closely adjacent to each other, and the lines of flux of these magnetic poles

penetrate the individual elements of the layer under a variety of angles ranging from perpendicular to the layer surface to parallel thereto.

The recording layer may suitably consist of a pulverulent mixture of hard magnetic and soft magnetic particles or grains, whereby the hard magnetic and the soft magnetic components may be adjusted with respect to their relative volumes so as to obtain the desired shielding effect. Preferably, the total volume of the soft magnetic particles will be greater than that of the hard magnetic particles so that the hard magnetic particles may be substantially completely covered by the soft magnetic particles. The two types of magnetic particles may be embedded in or bound together by means of a thermoplastic or thermosetting synthetic resin which melts or decomposes at a temperature above the range of working temperatures of the recording layer, or the magnetic particles may be attached to each other by sintering.

When a synthetic resin binder is used, it is desirable to have the highest possible filling ratio, in other words, the proportion of synthetic resin in the recording layer should be relatively small, because the total permeability drops significantly when the filling ratio is low. By forming the recording layer on rigid plates or, for instance, on printing cylinders which remain in the printing equipment, so that the recording layer need not possess a particularly high degree of resiliency, it is possible without difficulties to obtain a filling ratio of up to 80 percent which results in a total permeability which is sufficient for many purposes.

Such mixed magnetic layer may consist, for instance, of 30 percent by volume of Leguval a pourable polyester resin made by Bayer, 5 percent by volume of hardener, 45 percent by volume of Siemens 1500 N4 and 20 percent of volume of Bayer S 12. The mean permeability of this mixture, in cold condition, will be about  $\mu=15$ . The grain size of the highly coercive S 12 constituents preferably will be between 0.01 and 0.03 mm. in order to achieve the desired high resolution. The particle size of the highly permeable 1500 N4 constituent should be smaller by about one power of 10, i.e., between 1 and 3 microns. Due to the fact that the proportions by volume of the two components will be such that there will be between two and three parts by volume of highly permeable material for each part by volume of highly coercive material, it will be achieved that the highly coercive particles will be completely surrounded by the highly permeable particles.

A mixture such as described above will form a relatively rigid layer which may be cast on a printing cylinder or the like and the mean permeability of which and thus also the maximum shielding effect will be considerably reduced, due to the relatively high proportion of synthetic material having a permeability of  $\mu=1$ .

To increase the strength of the thus formed layer, it may be covered by a protective layer consisting exclusively of binder material. When a sintered layer is formed, the total permeability of the layer corresponds substantially to the total permeability of the magnetic starting materials since the organic binders, which are conventionally used for sintering, burn during the sintering process practically without leaving any residue.

Thus, a permeability of the layer which is close to the permeability of the highly permeable constituent can be obtained by adhering the magnetic particles by sintering. For instance, 60 percent by volume of 1500 N4 and 30 percent by volume of Bayer S 12 are mixed with 10 percent by volume of an aqueous solution of polyvinyl alcohol and the thus formed doughy mass is then pressed, for instance, by calendering into the desired shape, dried and heated throughout to between about 1000° and 1,200° C. The magnetic pigment S 12 produced by Farbenfabriken Bayer is a highly coercive, cobalt-containing cubical gamma- $\text{Fe}_2\text{O}_3$ .

It is thus possible to encase the hard magnetic particles in layers of soft magnetic material, preferably by sintering the soft magnetic particles. For this purpose, for instance, the permeable constituents may be finely comminuted by wet

grinding and mixed with the hard magnetic constituents which have a particle size which is preferably about 10 times greater than that of the permeable constituents and ranges between 0.01 and 0.03 mm. The thus formed mixture of hard and soft magnetic powders with a greater proportion by volume of soft magnetic material is then transformed into a deformable doughy mass or a liquid slurry by mixing with an organic solvent which is soluble in liquid solvents and which will burn below the sintering temperature of the magnetic particles, practically without leaving any residue. Polyvinyl alcohol, methyl cellulose, wax and the like are suitable for this purpose. If a doughy mass is formed in this manner, the same may be extruded and subsequently granulated. Preferably, the thus formed individual granules would have a diameter which is about twice the diameter of the hard magnetic particles since in this manner it is achieved that to the largest extent each granule contains only one hard magnetic particle. If a slurry has been formed, the same may be worked up by spray drying to form a mass of dried granules, whereby it is possible in conventional manner to control the size of the individual granules by suitably adjusting the conditions under which the spray drying is carried out.

It is then possible according to the present invention to form of the mass of individual composite granules, each consisting of a hard magnetic core and a soft magnetic covering, a coherent sintered layer. The temperatures required for forming by such sintered layer are considerably lower than those required for forming by sintering dense pressed bodies of the same material. In order to obtain a magnetic shielding effect, it will suffice if there is only a slight welding together of the contacting surface portions of the individual granules. This, for instance, may be achieved at 1,000° C., while for obtaining dense compressed sintered bodies of the same material a temperature of 1,350° C. would be required. At these temperatures and by choosing a suitable sintering atmosphere, the magnetic properties of the starting materials will not be affected.

If is furthermore proposed according to the present invention to embed the particles of magnetic materials in a resilient film of synthetic resin or in a fibrous layer, for instance a paper layer, or to apply the magnetic materials, particularly granules consisting of a hard magnetic core and a permeable cover layer, to an adhesive support. In this manner highly resilient storage means for magnetic recordings are produced which may be used, for instance as sound recording tape or as a magnetic direct copy of paperlike feel.

For embedding the magnetic granules in a fibrous material, methods may be used which are conventional in producing pigmented filter papers. For instance, the aluminum oxide paper No. 288 which is used for chromatographic purposes and produced by the firm of Carl Schleicher & Schuell may contain up to 40 percent of the inorganic pigment, whereby the pigment is incorporated into the paper pulp prior to forming of the paper web.

The magnetic recording carrier of the present invention can be produced in a particularly simple manner by sheathing or covering a hard magnetic wire which may form for instance a screen or a sieve, with a soft magnetic material.

Apart from the advantages in the production and mechanical properties of the carrier of magnetic recordings which consist essentially of covered particles or wires, i.e., particles or wires of hard magnetic material which are covered with soft magnetic material, there are also considerable advantages achieved in the use of the magnetic storage or recording devices of the present invention. For instance, it is possible to form raster layers of several types of covered granules or wires, whereby the different types will possess different specific magnetic properties. For instance, the magnetic recording carrier may consist of an even mixture of granules or wires the temperature dependency of the permeability of the covering layers of which may vary. Such storage means for magnetic recordings may also be used as a halftone raster since exposure to an infrared heat image will actuate all parti-

cles or wire portions only at the most intensively irradiated points.

Furthermore, if the hard magnetic core portions of the composite magnetic particles possess coercive forces of different strength, then a correlation between the intensity of radiation of the heat image and the magnetic field strength will be created which, as mentioned further above, may be used for producing colored halftone copies. A variation of the strength of the magnetization which is proportional to the intensity of the heat irradiation applied to the magnetic layer will also be achieved by surrounding the hard magnetic cores of the composite magnetic particles with a sheathing the permeability of which shows a linear dependency with respect to the temperature to which the storage device for magnetic recordings is exposed. This linear dependency may be such that the permeability is either increased or decreased upon exposure to rising temperatures.

If, according to a further embodiment of the present invention, the individual hard magnetic particles are covered with two different layers or sheathings the permeability of which shows a different temperature dependency, then it will be possible, for instance, upon forming a color copy from the latent magnetic image to achieve color selections which are independent from the temperatures selected for forming the magnetic image. This will be further described in connection with FIGS. 9 and 18.

According to another feature of the present invention, the coercive grains, with or without a sheathing of soft magnetic material, may be embedded in a layer of a material the permeability of which increases or decreases in a substantially linear manner with changes in the temperature to which the layer is exposed. This is particularly important when it is intended to achieve, in addition to a shielding of the hard magnetic grains, within certain temperature ranges a continuously changing effect of the external magnetic field within its effective range.

The selective effect of external field strengths of different values can be increased in a particularly advantageous manner by providing hard magnetic core grains which possess a different steepness of the slope of their respective initial magnetization curves of the well-known hysteresis loop. The selective effect of the sheathing can be increased by providing hard magnetic core grains which possess different Curie points, however, so that all of the different Curie points are within the range of working temperatures of the magnetic storage layer. In this case, there will be an upper and a lower limit of the actuating temperature for the individual composite magnetic particles.

According to another embodiment of the present invention, the magnetic materials, the magnetic characteristics of which differ in their temperature dependency, may be applied as a very thin layer, for instance, as a printed raster on the surface of a hard magnetic recording layer. In this manner a very thin composite recording layer or magnetic storage device can be easily produced. Composite layers of this type can be made so as to be highly heat sensitive particularly if, according to a further embodiment of the present invention, the surface layer is formed as a raster of alternately adjacently arranged highly coercive hard magnetic materials of relatively low permeability and of materials possessing a relatively high permeability which within the range of working temperatures of the magnetic storage layer is highly temperature dependent.

Due to the parallel arrangement of the low, constant, magnetic resistance particles with particles of high and temperature variable magnetic resistance, the degree of magnetization in a homogeneous magnetic field will vary proportional to the magnitude of the variation of permeability which are of the magnitude of about 3 Powers of 10.

Another advantageous arrangement according to the present invention provides that the surface of the magnetic storage device is to be formed of a raster arrangement of several permanently magnetizable materials possessing, respectively, different Curie points all of which are within the

range of operating temperatures of the magnetic storage means and, furthermore, preferably also having different coercive forces. In this manner a very simple magnetic storage arrangement can be provided which may be used for producing magnetic raster or screen prints or halftone copies.

The method of the present invention for using the magnetic storage means or layer provides, according to one embodiment, that a network formed of permanently magnetizable materials of low permeability and of materials of high, temperature dependent, variable permeability is exposed to a magnetizing or demagnetizing field.

According to another embodiment of the method of the present invention, the magnetic recording layer is to be magnetized or demagnetized at a temperature which is within the vicinity of the Curie point of the permeable portions of the recording layer, and is then to be read or scanned at the same or a higher temperature. In this manner the strength of the stored magnetic field of the data storage device of the present invention is fully utilized. If the magnetic storage layer includes several different permeable materials with different Curie points, then this method will permit by heating the data storage layer to different temperatures to obtain a selective scanning or radiation of the various groups of data or information which were incorporated in the data storage device at different temperatures.

Another embodiment of the method of the present invention provides that the storage device for magnetic recordings is magnetized or demagnetized at a temperature within the vicinity of the Curie points of the permeable portions of the storage layer, and is then scanned or read at a lower temperature. While thereby the outward effect of the initially applied magnetization will be of reduced strength, it will be achieved that the magnetic recording cannot be erased during reading or scanning of the same even if exposed to opposing magnetic fields of a strength which is a multiple of the strength of the magnetic field created by the recording.

A further embodiment of the method of the present invention provides that a heat image is formed of an original halftone image, which ranges over the operating temperatures of several permeable portions of the recording layer so that depending on the gray value or darkness of a respective portion of the original image, at the corresponding portions of the magnetic recording layer a different number of composite magnetic bodies (i.e., hard magnetic cores with a sheathing of a soft magnetic material of temperature dependent permeability) will be activated.

In this manner, it is possible without interposition of auxiliary means, particularly without interposition of an optical or chemical process, to convert a halftone image into a screen or halftone dot image wherein the variations in the color density of portions of the original image will be reproduced by the variations in the numbers of dots of uniform color density which will be formed per unit area. The fineness of the gradation as well as the steepness of the layer gradation can be controlled by suitably choosing the type and number of different components of the recording layer.

A raster which operates in a continuous manner like a photographic tone print raster or a halftone block, is formed by applying the heat image of an original image which shows a continuous gradation of gray values onto a layer of magnetic composite particles, the sheathing of which possesses a linear temperature dependency of its permeability, so that depending on the gray value of the respective portions of the original image, a rasterlike magnetic field of different densities will be formed at the corresponding portions of the magnetic recording layer. Since the dye or ink which is to be attracted by the latent magnetic image always possesses a certain threshold value, the magnetic field which extends from the individual composite magnetic grains will require a certain strength in order to be effective at a sufficient distance from the magnetic grain from which it emanates in order to achieve that no gap in ink or dye attraction appears between adjacent composite

magnetic grains. Thus, upon a low degree of magnetization, the individual magnetic raster grains will either attract no ink at all or will attract ink only over a very limited area which may be less than the surface area occupied by the respective composite magnetic grain. If the field strength of the permanent magnetization is low, a gap will be formed in this manner which is or relatively light color or color intensity and which will consist of fine ink points spaced from each other, while at portions of the magnetic image from which a greater magnetic force or field strength emanates, the individual areas of attraction will grow together and thus a continuously inked copy portion will be formed.

The method of the present invention also provides that the magnetic storage layer is exposed to the heat images of several color separations of a colored original image, which heat images contact the magnetic storage layer with different intensities. In this case, the sheathings of the individual composite magnetic grains will be of different temperature dependency of their permeability and, in addition, the permanently magnetizable core portions of the composite magnetic grains may possess different Curie points. Differently colored dyes or printing inks are then exposed to and attracted by the thus formed latent magnetic image at different temperatures of the magnetic recording layer, whereby, in the case of this magnetic image carrier one has to start with the lowest temperature range.

According to this method at a given temperature only those composite or sheathed magnetic grains will be magnetized for which the temperature range between the Curie point of the sheathing material and the preferably higher Curie point of the core material corresponds to the intensity of the respective color separation. Composite magnetic grains with a higher Curie point of the sheathing are still blocked, while grains with a lower Curie point will respond but will not be able to maintain their magnetization. The application of the color separations to the recording layer, i.e. the exposure of the recording layer to the heat images of the color separations must start with the color separation of highest intensity since upon exposure of the recording layer to a higher temperature range latent magnetic images which are formed previously thereto within lower temperature ranges will be extinguished. Since the conventional original colored images such as images on a paper support or transparencies do not possess complete coverage even at the darkest image portions and since furthermore, the blocking effect of the corresponding radiating energy does not depend directly on the color of the respective image portions, it is always possible to transpose each color separation by suitable choice of the radiant energy such as a source of infrared radiation, into a heat image within a temperature range which does not or only slightly overlaps the temperature ranges of the heat images formed of the other color separations.

In order to form a color copy from the latent magnetic image, the magnetic storage layer is evenly heated to the average or mean actuating temperature of one of the groups of composite magnetic particles, starting with the group which is actuated within the lowest temperature range, and the dye or ink of the color corresponding to this temperature range is then exposed to the magnetic storage layer so as to be attracted only by the thus activated composite magnetic grains. All groups of magnetic grains which will emanate magnetic force at higher temperature ranges are still blocked while all groups of composite magnetic grains which are activated at lower temperature ranges are already extinguished. Consequently, a magnetic ink which is evenly exposed to the thus heated magnetic storage layer will be attracted and attach itself only to the group of composite magnetic grains, the latent image of which corresponds to a single color separation.

In this manner, it is possible to make color copies of a colored transparency on paper layers in which the composite magnetic particles are sufficiently fine or of sufficiently small diameter, and it is possible to reproduce mixed colors in this manner.

According to a further embodiment of the present method, the heat images of several color separations of a colored original image are applied with different intensities to a magnetic recording layer which contains permeable constituents of linear temperature dependency of their permeability and/or permanently magnetizable constituents of different coercive force, and/or different temperature dependency of the permanently magnetizable constituents and/or their sheathings, so that each color will be correlated to a certain range of magnetic field strength.

This latent stored image of the color image to be stored, which is proportional to the field intensity, can now be used to produce thereon in different ways a color copy of the original color image. For instance, the individual magnetic printing inks may be exposed to the magnetic recording layer carrying the latent image at different distances therefrom, or the individual magnetic printing inks may be of different permeability and may be exposed to the magnetic storage layer at one and the same distance therefrom possibly in the form of a dispersion.

For instance, a recording layer carrying a latent magnetic image consisting of portions of different field intensity of strength may be passed successively along inking arrangements or rollers located at different distances or forming air-gaps of different length with the magnetic recording layer, so that at first the magnetic ink located the shortest distance from the latent magnetic image is exposed to the same. In this manner, magnetic ink will be applied to the latent magnetic image successively from all ink rollers which are located at a distance from the magnetic recording which still can be overcome by the magnetic field strength of the respective portion of the latent magnetic image. If magnetic inks of high covering power are to be applied, whereby preferably the color with lowest covering power, for instance, yellow is correlated to the lowest magnetic field strength or intensity, and the color of highest covering power, for instance, black, is correlated to the highest magnetic field strength, the inking arrangement which is last actuated will determine the final color of the respective portion of the inked recording layer.

When it is desired to produce a copy of the latent magnetic color image which is to be transferred to another image carrier, for instance a paper sheet, then the application or attraction of colored magnetic ink must be started with the ink supplied by the inking arrangement which forms the largest airgap with the magnetic recording layer. This is necessary in order to achieve that the dyes which are actuated only by portions of the recording layer will form an outer or upper layer of the thus produced color print. Any desired number of color copies or prints can be thus produced since the latent magnetic image of the recording layer is not destroyed thereby.

When colored copies of the original image are to be produced with magnetic dyes or printing inks of different permeability, then the length of the airgap between each of the dye supplies or inking arrangements and the magnetic storage layer may be the same for all colors, or all of the different colored magnetic inks or dyes may be jointly offered in the form of a dispersion. The dye with the greatest magnetic permeability will then be attracted by the portions of the magnetic recording layer creating the lowest field intensity, while the dye of lowest permeability will be only attracted by the portions of the magnetic recording layer creating the highest field intensity. In both cases, the color characteristics of the visible color copy can be influenced by adjusting the minimum field intensity at which the individual magnetic inks are attracted. This can be done by changing the distance from which the magnetic ink is supplied or offered or exposed to the magnetic storage layer carrying the latent image.

Apart from these inking methods which operate depending on a minimum field intensity and according to which each portion or point of the magnetic storage layer will attract a number of different magnetic inks, which number depends on the final color of such point or portion, the present invention also proposes an inking method for producing colored copies

according to which the individual inking arrangement for any given color will not dispense magnetic ink below or above a certain range of magnetic field intensity or strength. This is accomplished by exposing the individual magnetic inks to the magnetic recording layer either on a permeable support or through a permeable orifice, the magnetic saturation value of which is lower than that of the respective ink by at most the threshold value of the respective inking arrangement, and which support or orifice, prior to reaching the saturation value of the ink has a lower total permeability than the latter.

With inking devices of this kind, like those described further above, there exists a threshold value which depends on the permeability of the magnetic ink or dye and the distance of the magnetic dye from the magnetic recording layer carrying the latent image. Below this threshold value the magnetic dye will not be attracted. Since at the beginning the total permeability of the dye is higher than that of the support, the induced magnetization within the dye rises faster than the opposing field induced in the support. As soon as the difference between these two magnetizations become greater than the threshold value of the inking device, dye will be supplied to or attracted by the magnetic recording layer. When the inking arrangement is exposed to external magnetic fields of a greater strength than the saturation value of the magnetic ink, then with increase of the external field only the induction of the permeable support will be increased and the difference in the magnetization will be reduced so that at a certain strength of the external field this difference will fall below the threshold value of the inking arrangement.

Thus, every point or portion of the magnetic recording layer will be supplied by this inking arrangement only with the specific magnetic ink which is correlated to the intensity of the magnetic field created by such point or portion. It is possible thereby to shift the range of magnetic field strength or intensity at which the inking arrangement for the specific colored ink will be actuated, by applying a permanent magnetic field which is superposed upon the magnetic field of the magnetic printing form or layer carrying the latent magnetic image.

According to a further embodiment of the present invention, the individual colored inks are offered by means of inking arrangements having partially overlapping range responses.

In this manner a subtractive mixed color application can be carried out. Magnetic printing methods are particularly suitable in this respect because it is possible to carry out the ink transfer without contact between the inking arrangement and the support for the transferred ink such as a copy sheet and thus even in the case of the so-called "wet-in-wet" printing process contamination of the not yet applied dye at the inking arrangement, which would severely interfere with the subtractive method, will not take place.

On the other hand, particularly when very weak latent magnetic images are used for forming the copy, it might be advantageous to apply the magnetic ink with contact between the ink supplying roller and the printing form and to wet the latter in the manner conventionally carried out in connection with a planographic or lithographic printing methods in order to avoid transfer of ink by adhesion at the nonmagnetic portions of the printing form, i.e. at the portions of the printing form which are not within a magnetic field of the required strength. For this purpose, preferably an ink is used which, like an offset oil, consists of a binder which will be absorbed by the printing form, for instance a paper sheet, and which binder contains a large proportion of magnetic particles and pigment particles and/or magnetic pigments.

The field strength method may be carried out in connection with all recording layers consisting of portions or particles on which different magnetic field strengths can be imposed dependent on the intensity of the radiant heat image to which such recording layer is exposed. Thus, for instance recording layers may be used which contain permanently magnetizable, premagnetized constituents of different coercive force and different Curie points, or permanently magnetizable con-

stituents of different coercive force surrounded by sheathings of a different temperature dependency of their permeabilities. Furthermore, it is also possible to use in a simple manner a combination layer comprising one material with linear temperature dependency of its magnetic characteristics having embedded therein magnetizable core portions which have a Curie point located above the operating temperature of the recording layer. The large ranges of magnetic field strengths corresponding to a color may then be adjusted by suitably choosing different initial magnetic field intensities during magnetization, while the smaller differences in the magnetic field strength within the range of a color which determine quantitatively the strength or amount of the respective color which will be attracted, can be adjusted by means of the linear temperature dependency of the permeability of the covering layer or sheathing of the individual core portions. The foregoing will be further described in connection with FIGS. 14 and 15 of the drawing.

By using these layers, several color separations may be united with each other on a single printing form and may be supplied with magnetic ink in one path along inking arrangements for different colors which will be activated depending on the respective magnetic field intensities, and then transferred from the printing form onto a copy sheet, and this process may be repeated as often as desired since the magnetic printing form or the latent magnetic image will not be affected thereby. Since with respect to these layers the selection of temperatures during formation of the magnetic image acts only in one direction so that recordings applied with varying intensities will partially be superposed upon each other, the methods which can be carried out therewith are predominantly suitable for the reproduction of screened or rastered colored original images or form multiple form printing with changes in the printed matter or information of different forms within each set, whereby each portion of the surface of the magnetic recording layer will serve only for the recording of a single pure or primary color.

For the halftone block reproduction of mixed colors of an original image which is not a screened or rastered image, and without interposition of optical or chemical screening processes, a preferred embodiment of the present invention provides that during application with different intensities of the heat images of the individual color separations of a multicolor original image external magnetic fields of different field strengths are to be applied.

Thereby, preferably, the strength or intensity of the external magnetic field should be inversely proportional to the intensity of the heat image of the respective color separation. Thereby a double selection can be achieved, on the one hand, based on the release temperature and, on the other hand, based on the magnetic field strength. If then the ranges of magnetic field strength or intensity of the individual groups of magnetic particles responding to the different colors are arranged without overlapping or if the composite magnetic particles contain cores of differently steep slope of their respective initial magnetizing curves, then the magnetic field strength which is correlated with the magnetic particles of low coercive force cannot effectively magnetize the particles of higher coercive force, while the particles of lower coercive force are protected by the blocking effect of the sheathing which blocking effect will terminate only at higher temperatures. In this manner it is possible to dissociate or divide even mixed colors into networks or rasters of magnetic particles which represent the individual color components.

According to another embodiment of the present invention, the above-described storage devices for magnetic recordings or carriers of latent magnetic images can be utilized in a simple manner for multiple form printing with changes in the printed matter or information within different forms of each set. This can be accomplished by forming a plurality of latent magnetic images each of which, however, does not represent the heat image of a color separation but a specific information or printing arrangement, and each of which is imposed upon

the magnetic image carrier or storage device at a different temperature so that the latent image can be read or utilized with a temperature selective arrangement or an arrangement which is selective with respect to the magnetic field strength.

5 It is possible in this manner, for instance by selecting different reproduction temperatures or magnetic field strengths to print a set of multiple forms consecutively, starting from printing minimum information, for instance for a delivery slip, up to the complete text, for instance a bill including address, price, discounts, etc. It is also possible with the help of selecting maximum-minimum ranges of magnetic field strength to print or delete individual lines or columns, for instance of a work ticket.

Furthermore, according to another embodiment of the 15 method of the present invention it is also possible to selectively reproduce portions of information or of a latent magnetic image although the entire latent magnetic image has been formed in a uniform manner. This is possible by forming the latent magnetic image in a layer or the like which includes

20 constituents the permeability of which is temperature dependent and by heating certain lines or other portions of the magnetic image carrier to a temperature at which the blocking effect of the particles of temperature dependent permeability is greatly reduced. An inking arrangement having a threshold

25 value of about the magnetic field strength of the not released, i.e., still blocked particles will then cause only transfer of ink corresponding to the released particles or magnetic image portions. It is possible with this arrangement, independent of the number of different magnetic components in the recording layer, to reproduce any desired number of individual portions of an original image, including relatively very small portions of such image.

It is particularly advantageous to form the heat image to 30 which the magnetic recording layer is to be exposed by heating the original image with a source of infrared rays and to shield portions of the original image which upon copying should be free of ink.

According to a further embodiment of the present invention, the arrangement for producing copies from a latent magnetic image will include for each differently colored magnetic ink or dye which is to be applied an ink supply roller or screen roller which consists essentially of a ferromagnetic material having a value of magnetic saturation which is lower than that 40 of the magnetic ink by at most the threshold value of the dye or magnetic ink dispenser, and which prior to reaching the saturation value of the magnetic ink has a lesser total permeability than the latter. Preferably in such arrangement, the distance of each ink applying roller or screen from the carrier 45 of the latent magnetic image should be individually adjustable.

Referring now to the drawing and particularly to FIG. 1, it is noted that the temperature dependency of the permeability of the mixed ferrites  $Ni_{0.3}Zn_{0.7}Fe_2O_4$ ,  $Ni_{0.35}Zn_{0.65}Fe_2O_4$  and  $Mn_{0.5}Zn_{0.5}Fe_2O_4$  are taken from the treatise "Ferrite" by Dr. J.

55 Smit and Dr. H. P. J. Wijn, published in "Philip technische Bibliothek," 1962. The first two mentioned materials belong to a series of materials within which the temperature dependent properties can be continuously changed depending on the proportion of the nickel and zinc constituents. "1500 N4."

60 is the trade name of a ferrite which is offered by Siemens & Halske AG for use in high-frequency cores. It is a nickel-zinc ferrite of the approximate composition  $Ni_{0.35}Zn_{0.65}Fe_2O_4$  and has an initial permeability at room temperature of  $\mu=1,500$ . "Thermoperm" is a trade name of an iron nickel alloy made

65 by Krupp, containing about 30 percent nickel and used for temperature compensation in magnetic circuits.

Ambient room temperature is indicated by  $A$  and the temperature at which the respective material reaches its maximum permeability by  $B$ . The temperature at which the 70 permeability has just dropped to the value 1 of a nonmagnetic material is indicated by  $C$ . This temperature is the approximate equivalent of the Curie point or temperature. It can be seen that the heating of the ferrite materials from  $A$  to  $B_1-B_4$  will cause an approximately linear rise of the permeability by about the factor 1.5.

In the case of "Thermoperm," the permeability curve slopes downwardly in a linear manner at a factor of about 100, while further heating of the ferrites from the respective points *B* to the respective points *C* causes a drastic linear drop of the permeability by about the factor 1,000 down to the value 1 of a nonmagnetic material. When these ferrites form part of a mixed magnetic layer according to the present invention, then, as will be described in detail below, the shielding of the hard magnetic coercive constituents against an external magnetic field, as well as the weakening of the outwardly extending magnetic field emanating from these coercive constituents will change within the corresponding temperature ranges by about the same factor.

FIG. 2 is a graphic illustration of the temperature dependency of the lowering of a saturation premagnetization of several chromium oxides which are known from the patent literature and which, for instance, are described in German published application 1,152,932. In this case it is also possible to distinguish a temperature range from room temperature *A* to temperatures *B*<sub>6</sub>-*B*<sub>9</sub> wherein the premagnetization is slowly reduced by about the factor 1.5, as well as a further range up to the temperatures *C*<sub>6</sub>-*C*<sub>9</sub> wherein the premagnetization disappears completely.

If one of these magnetic materials is used as the coercive constituent of a mixed magnetic layer according to the present invention the permeable constituent of which loses its permeability below one of the temperatures *C*<sub>6</sub>-*C*<sub>9</sub>, then a layer is formed which can be magnetized only within a closely limited temperature range.

On the other hand, if the mixed layer consists only of premagnetized coercive or hard magnetic constituents having different Curie points, for instance of two materials the Curie points of which are at *C*<sub>7</sub>-*C*<sub>9</sub> and if different colors, for instance red and black are correlated to the different coercive forces of these materials, then heating from *A* to *B*<sub>7</sub> will first cause a dropping of the premagnetization and consequently of the intensity of red inking by about the factor 1.5. Upon further heating, the premagnetization will drop suddenly to the magnetic field strength correlated to the black magnetic ink and will finally disappear completely at *C*<sub>9</sub> after first dropping to *B*<sub>9</sub>, which would correspond to a white portion of the pattern or original image.

FIG. 3 is a schematic view of the structure of a mixed layer according to the present invention which is formed of soft magnetic constituents 1 and hard magnetic constituents 2. The soft magnetic constituents may consist for instance of the ferrite  $Mn_{0.5}Zn_{0.5}Fe_2O_4$  which has been shown in FIG. 1 and which at 120° C. has a permeability of about  $\mu=2,000$  while at 130° C. the permeability has dropped to the value 1 of a nonmagnetic material. As the hard magnetic constituents, for instance the magnetic pigment known under the trade name "Bayer S 12" may be used, i.e., a highly coercive, cobalt-containing cubical gamma- $Fe_2O_3$  having a coercive force of about 800 Oersted and within the range of operating temperatures of the layer a nearly unchanging permeability of  $\mu=10$ .

According to FIG. 4, hard magnetic wires or grains 3 which may consist for instance of Bayer S 12 are covered with a soft magnetic sheathing or covering 4 which may consist for instance of the above-described  $Mn_{0.5}Zn_{0.5}Fe_2O_4$ . The wires may be arranged in the form of a screen or sieve or, as illustrated, the wires or grains may be embedded in a nonmagnetic carrier layer consisting for instance of resilient synthetic material, which, as far as magnetic properties are concerned, will have the same effect as if the materials 3 and 4 were embedded in air.

For instance, as described further above, 60 percent by volume of 1,500 N4 may be wet ground in a ball mill for between about 20 and 40 hours until the particle size has been reduced to between 1 and 3 microns. A doughlike mass is then formed by mixing with 30 percent by volume of Bayer S 12 having a particle size of between about 10 and 30 microns and 10 percent by volume of an aqueous solution containing about 12 percent polyvinyl alcohol. The thus formed dough is then

pressed through a perforated plate the perforations of which have the diameter of the desired grain size so as to form strands of such diameter and these strands are then comminuted for instance with a chopping knife. The diameter and length of the thus formed cylindrical particles are so chosen that they are equal to somewhat less than twice the diameter of the hard magnetic Bayer S 12 particles. It is achieved in this manner that each of the thus formed composite grains contains only one highly coercive permanently magnetic particle.

A suspension which may be spray dried can be formed of 50 percent by volume of an aqueous solution containing about 3 percent polyvinyl alcohol, 30 percent by volume 1,500 N4 and 20 percent by volume Bayer S 12.

Spray drying is carried out in conventional manner substantially similar to that used for producing milk powder. The suspension is mixed with air and sprayed through fine nozzles under high pressure into a stream of hot air which, in countercurrent to the sprayed suspension, withdraws moisture from the latter. The grain size of the thus formed granular mass depends on the viscosity of the suspension, the diameter of the nozzle orifices and the applied air pressure.

The thus obtained granular mass is then sintered by heating at about 1,000° as described further above. Since thereby, in contrast to the first-described method of forming strands of the material, the granular mass is not compressed, the individual grains will remain substantially separated. Should some of the grains bake together, they can be easily separated again by impact comminution for instance in an impact mill. The sintered bodies are now rolled into a thermoplastic synthetic material, for instance into soft polyvinyl chloride and then together rolled to form a thin foil such as illustrated in FIG. 4, wherein the soft polyvinyl chloride forms the carrier layer 5.

On the other hand, it is also possible to embed the composite grains 3-4 in finely subdivided iron-nickel powder, for instance Thermoperm and to sinter the thus formed mixture. In this case, carrier layer 5 of FIG. 4, consisting of Thermoperm, would be of a linear temperature dependency of its permeability with lower permeabilities at higher temperatures as illustrated in FIG. 1.

Furthermore, FIG. 4 may also be considered as a cross-sectional view through a sieve or screen of a hard magnetic wire 3 which is coated with a soft magnetic material 4, in which case the surrounding layer 5 would represent nothing but air.

A thus covered wire can be drawn in conventional manner from a cylindrical bar of soft magnetic material having a hard magnetic core and substantially the same ratio between the diameter of the hard magnetic core and the soft magnetic outer bar as the ratio between these diameters in the drawn wire.

A layer of individual composite magnetic grains can be produced by applying the sintered composite grains by means of an adjustable rake to an adhesive support, for instance the gum-arabic coated surface of a sheet of paper.

FIG. 5 shows a preferably magnetically neutral carrier layer 6 to which has been applied a screen or raster of hard magnetic particles 7 and soft magnetic particles 8 which may consist of the above-described magnetic materials.

The structure of FIG. 4 can be produced in conventional manner, for instance similar to the method by which magnetically readable checks are produced with printing inks containing magnetic inks. Instead of indicia such as numbers, in the present case a fine dot or dash raster or screen is imprinted whereby a highly permeable pigment for instance 1500 N4 is applied so as to fill the voids in a printed screen of highly coercive pigment, for instance Bayer S 12.

According to one embodiment of the present invention, permanently magnetizable chromium oxides of the type illustrated in FIG. 2 may be used as the magnetic pigments, for carrying out a method, as described further above, wherein the mixed magnetic layer consists only of premagnetized coercive constituents having different Curie points.

In the left half of each of FIGS. 3, 4 and 5, the approximate course of the lines of magnetic force of a homogeneous external magnetic field are shown which penetrate through the respective layer at a temperature which is below the Curie point of the soft magnetic portions 1, 4 and 8, respectively.

The right half of each of FIGS. 3, 4 and 5 shows the course or path of the lines of magnetic force at a temperature above the above-mentioned Curie point, such as in the case of the materials of FIGS. 3-5, a temperature above 130°C.

As long as the permeability of the soft magnetic constituents 1, 4 and 8 which at most might have a value of 2,000 amounts to a multiple of the permeability of the hard magnetic constituents the permeability of which has a value of about 10, the hard magnetic constituents will remain nearly field free. However, as soon as the permeability of the soft magnetic constituents has dropped to the value 1 of nonmagnetic materials, the lines of magnetic force will favor passage through the hard magnetic constituents.

The distribution of the magnetic field in a substantially two-dimensional screen or raster according to FIG. 5 can be computed in accordance with the laws applicable to an electrical network whereby the electric resistance is to be replaced by the magnetic resistance, the latter being proportional to the reciprocal value of the permeability. In the case of a three-dimensional lattice, an increased shielding effect will be found due to the bending of the lines of magnetic force at the separating planes between two media of different permeability. For instance, for a spherical shell such as a hard magnetic particle covered by soft magnetic material, the following equation according to R. Gans "Einfuehrung in die Theorie des Magnetismus," published by Teubner, 1908, will apply:

$$(1) \quad H^* = \frac{1}{1 + \frac{2}{9} [(\mu - 1)^2 / \mu] \cdot \left[ 1 - \left( \frac{r_i}{r_o} \right)^2 \right]} \cdot H$$

wherein  $r_i$  and  $r_o$  indicate the inner and outer radius of the spherical shell of soft magnetic material.

It is thus possible to calculate a shielding factor which connects the inner magnetic field  $H^*$  unequivocally with the outer or external field  $H$ . The formula applies strictly only for a permeability 1 of the material located inside the shell. For a permeability of the highly coercive hard magnetic core portion which is equal to about 10, the formula must be appropriately adapted.

By choosing suitable proportions between core diameter and outer diameter of the composite magnetic particle, and/or between the permeabilities of the core and the covering layer, any desired shielding factor may be obtained which, furthermore, can be changed in a well-defined manner by adjusting the temperature of the layer, due to the temperature dependency of the respective permeabilities.

FIG. 6 illustrates four different core particles 9-12 which have different Curie points or temperatures indicated in core particle 12 as  $T_c$ , and different remanences of saturation. Each of the core portions 9-12, respectively is surrounded by covering or sheathing 13-16, respectively and the materials of coverings 13-16 have different temperature dependencies of their permeability. For instance, a chromium oxide according to FIG. 2 may serve as core, while the covering layer or sheathing may be formed of a material of the composition  $Ni_xZn_yFe_2O_4$ , in accordance with FIG. 1. All of the composite magnetic particles are embedded in a soft magnetic layer 17 of linear temperature dependency of its permeability, similar to that of the Thermoperm of FIG. 1.

The composite magnetic particles of FIGS. 6, 14 and 18 may be produced in a manner substantially similar to that described in connection with FIG. 4, with suitable replacement of the specific magnetic materials.

FIG. 7 relates to FIG. 6 and shows on a uniform temperature scale the permeability curves  $m13$  to  $m16$  of the sheathings or core coverings 13 to 16, the magnetization curves  $k9$  to  $k12$  of the cores 9 to 12 and also the linear permeability curve 1 of the embedding material.

If a different color is correlated to each of the different types of composite magnetic grains, then it is only necessary to see to it (as will be described in more detail further below) that each color separation is applied to the recording layer as a heat image within a predetermined temperature range so that only the grains which are correlated to this color will be magnetized by an external homogeneous magnetic field the strength of which should be above the value of magnetic saturation of the grain type having the highest coercive force. For instance, within the temperature range of between 80° and 90° the "blue" and the "black" grains are still blocked due to the characteristics of the permeability curves  $m15$  and  $m16$ . The blocking of the "yellow" grains has been terminated due to the drop of the curve  $m13$  as well as the blocking of the "red" grains due to the drop of the curve  $m14$ . However, the "yellow" composite grain can no longer be subjected to permanent magnetization since the material of the core of the "yellow" grain has already been heated beyond its Curie point, as indicated by curve  $k9$ . Thus, within the temperature range of between 80° and 90°, only the "red" grains are subjected to permanent magnetization, whereby due to the fact of the linear temperature dependency of the permeability of the embedding layer 17, a gradation of the intensity within the red range will be achieved. Similar considerations are applicable for all of the various types of composite magnetic grains whereby the grain type which is correlated to the highest temperature range, in the present case the "black" composite grains may have any desired Curie point since it is to be actuated at all temperatures which are higher than the release temperature of the permeability curve  $m16$  of its covering layer. Below the release temperature of the permeability curve  $m13$  none of the composite grains of FIGS. 6 and 7 will be magnetized. At such portions no color will subsequently be applied to the latent magnetic image so that at such portions the color copy will be of the color of the supporting sheet, for instance white if the color copy is produced on a white paper sheet.

Referring now to FIG. 8, it is shown how the individual colors can be offered to the recording layer from different distances, provided that the various portions of the recording layer are of different magnetic strength in correlation to the individual colors, as described in connection with FIGS. 6 and 7. The field strength of the composite magnetic grains 12-16 which are correlated to the black color and which, according to the present example, amounts of 200 Oerstedt, will then be capable with respect to all color supply rollers 18 to 22 to overcome the adhesion of the ink film at the roller as well as any other retarding forces of the ink or dye. Since, however, black has been applied as the last ink, and assuming that opaque, covering inks have been applied, the outward appearance of the respective portion of the reproduced image or of a paper support interposed between the magnetic recording layer or printing form and the ink supply rollers on which the copy of the image is formed, will be black. If the visible image which is formed is to be further transferred from its original support to a final support, then the visible image must be formed by passing the magnetic recording layer or initial support along the ink supply rollers in a direction opposite to that of arrow D so that initially the color black will form the lowermost ink layer and only upon transfer onto the final support, the opaque black ink portions will appear on the visible surface. In carrying out this process care should be taken by suitably choosing the printing form surface, by wetting or by utilization of a separating agent, in a manner known per se in the art, that the ink, under the influence of the respective magnetic field will be transferred as a coherent film.

The "blue" composite grain, due to its lower coercive force of only 130 Oerstedt will only be capable to attract ink from ink rollers 19 to 21, the distances  $d1$  to  $d3$  between roller and magnetic recording layer being smaller than the distance  $d4$  of ink roller 18. Blue will then be the topmost color or, by reversing the direction of passage of the recording layer relative to the ink rollers, blue will be the bottom color, and this will be desired if the color image formed in this manner for in-

stance on the recording layer is to be transferred onto another support. Every composite grain which during application of the latent magnetic image was not subjected to permanent magnetization, will not attract any of the inks from the various ink rollers and thus, in the case of a white support for the visible color reproduction may be considered as "white" grain 22.

It is, of course, also possible in the same manner to imprint different data or sets of information instead of different colors, for instance when it is desired to carry out multiple form printing with changes in the printed matter of different forms of each set. In this case, the portions of the support to which ink is supplied from the individual inking arrangements or ink supply rollers should not overlap each other.

The same effect which is achieved by arranging the various ink rollers at different distances from the magnetic recording layer carrying the latent magnetic image can also be achieved by using magnetic inks of different permeability. In this case, all of the ink rollers may be arranged at the same distance from the recording layer. In both cases, the required strength of the magnetic field and, due to the retarding forces within the magnetic ink, also the strength of intensity of the individual ink applications can be controlled by adjusting screws 23. Adjusting screws 23 are arranged in a frame member 24 or the like of the inking arrangement and coact with a slot 25a of a bearing block 25 for the respective ink roller, which bearing block is guided in a slot 26.

As illustrated in FIG. 9 the visible color image can also be produced in such a manner that each differently colored magnetic ink is offered to or attracted by the magnetic recording layer carrying the magnetic image only at a certain temperature. For instance, if the recording layer according to FIG. 6, is heated, as shown in FIG. 9, by means of a heat source 27 to a temperature of 70° C. and then passed along yellow ink supply roller 21, only the "yellow" composite magnetic grains which are already deblocked at this temperature will accept ink. After further heating by means of a heat source 27 to 80° C., the latent "yellow" image will be extinguished due to the fact that the Curie point of the core portion of the "yellow" recording or grain has been exceeded while the "red" composite grains will be deblocked by exceeding the Curie point of the covering layer or sheathing of the "red" grains so that only the "red" grains will attract ink from red ink supply roller 20. In similar manner, the other types of composite grains can be successively deblocked and subsequently their latent image extinguished by successively raising the temperature to which the magnetic recording layer is exposed.

By supplying ink in the last-described manner it is not necessary that the different types of magnetic core portions possess different coercive forces since only the difference in their Curie points is utilized.

As shown in FIGS. 10-12 it is also possible to supply selectively differently colored inks to the recording layer or a copy sheet without requiring opaque inks of high covering qualities and without destroying the latent magnetic image during formation of the visible color copy. This is accomplished by supplying the ink through a ferromagnetic screen 28 (FIG. 11) or on a ferromagnetic ink supply roller 29 (FIG. 12) whereby the total permeability of screen or sieve 28 and roller 29 has to increase at a slower rate than that of the magnetic ink and whereby, however, the value of magnetic saturation of the screen or roller will be lower than that of the magnetic ink by at most the threshold value of the inking arrangement.

According to FIG. 10, the ink may consist for instance of the material known under the trade name "Permalloy 78" and the inking roller 29 or the screen 28 of the material known under the trade name "Sinimax" or these materials may be at least admixed to the ink and the ink supporting roller or screen.

Generally, the materials which are utilized in accordance with the embodiments of FIGS. 10, 11, 12 and 17 can be found in "Permanent Magnets and Their Applications" by Parker and Studders, published by John Wiley & Sons Inc., New York-London 1962, and attention is particularly directed

to FIG. 4, 30 between pages 152 and 153, and the tables on pages 148 and 149.

It may be assumed that a ferromagnetic screen 28 formed of Sinimax is arranged according to FIG. 11 at the same distance from the latent magnetic image or the magnetic recording layer as the magnetic ink which consists of Permalloy 78. The magnetization of both mentioned materials by the latent magnetic image or the magnetic field created by recording layer 17 will then correspond to the curves shown in FIG. 10 whereby the ink, until it reaches its magnetic saturation value will be more strongly magnetized than the material of which the screen 28 is formed. Since the magnetic ink particles 30, on the one hand, are attracted by the magnetic field of the latent magnetic image but, on the other hand, are held back by the field formed by induction in screen 28, and also by the ink's inherent cohesive forces, attraction of the ink by the recording layer will take place only if the induced magnetic force of the ink is greater by a certain value than the induced magnetic force of the screen. This limit of response is indicated in FIG. 10 by the line a—a. Thus, attraction of the ink by the magnetic recording layer or the latent magnetic image will take place only within the crosshatched area, i.e. between a minimum field strength b and a maximum field strength c. This effect may be utilized not only for multicolor printing but also in connection with multiple form printing with changes in the printed matter of different forms of each set.

As soon as the magnetic saturation value of the ink has been reached, a further increase in the strength of the external magnetic field will only serve to increase the holding forces or the internal magnetic field of the screen or roller until the value of magnetic saturation of these elements has been reached. Lifting of the ink from the roller or passage of the ink through the openings of the screen can also be prevented at any desired increase of the external magnetic field, if the magnetic saturation value of the base is equal or at most smaller by the value d than the saturation value of the ink. If there is a difference in the distance between the recording layer and the ink on the one hand and the supporting roller portion 29 on the other hand, as shown in FIG. 12, this will correspond in the representation of FIG. 10 only to an apparent change in the scale of the ordinate in accordance with the dot-dash line of the Sinimax permeability curve. The saturation values and thus the basic principle of this arrangement are not affected thereby.

In order to create additional ranges of magnetic field strengths, further combinations of suitable materials can be arranged, or the range of response of the combination of materials described in FIGS. 10-12 can be shifted to any desired part of the ordinate of FIG. 10 by providing corresponding opposing magnetic fields. Such opposing magnetic fields may for instance emanate, in accordance with FIG. 12, from a tubular radially magnetized permanent magnet or from a corresponding, possibly adjustable electromagnet which is interposed between the core portion 31 and the surface layer 29 of the ink roller of FIG. 12.

Since for the selective inking based on variations of the magnetic field strength it is not necessary to provide different distances between the inking arrangement and the recording layer or latent magnetic image, it is also possible to operate in this manner with very weak latent magnetic images, particularly by direct contact between the ink supplying roller and the recording layer or printing form. In this case it is advantageous to wet the magnetic printing form like an offset printing form in order to eliminate adhesive forces between the ink and the surface of the printing form. The ink will then pass from the ink supply roller only to the correspondingly magnetized portions of the recording layer or printing form, notwithstanding the direct contact between the latter and the ink supply roller. The printing ink which is to be used in the presently described embodiment of the present invention, preferably will consist essentially of a binding agent which like an offset oil penetrates a paper support or copy sheet and in which as high as possible a proportion of magnetic particles

and pigments or of magnetic pigments such as black ferrites is incorporated. Experiments have shown that the binding agent attaches itself to the magnetic particles and is carried along by the latter with great force onto the paper copy sheet. On the other hand, the binding agent which penetrates into the paper will carry along magnetic pigment particles. The attachment of the binding agent to the magnetic pigment can be further improved by providing the pigment particles with a fat attracting covering consisting for instance of polyvinyl alcohol.

The arrangement shown in FIG. 6 may be modified and also simplified in various ways. For instance, it is possible to operate without requiring that the Curie point of the magnetic core portion must be within the range of operating temperatures, provided that halftone block images are to be recorded in which each point represents only one basic color. In this case, it is also possible to replace the carrier layer 17 of linear temperature dependent permeability with a synthetic material or paper in which the composite magnetic grains are embedded. Such halftone images can also be reproduced with a layer which contains sheathed or covered magnetic cores of different Curie points and different values of magnetic saturation.

In this case, the cores need only be premagnetized and step-wise demagnetized by being subjected to different degrees of heating in areas corresponding to the different characteristics of the original image.

There exists the further possibility to utilize only one type of permanent magnetic core portions combined with sheathings or coverings the temperature dependency of the permeability of which varies between different groups of the thus formed composite magnetic grains. Upon forming a negative heat image of an original image which has a continuous gradation of its color intensities, so that portions of varying intensity extend over the entire heat responsive range of for instance four of such coverings of different temperature dependency of their permeability, it will be achieved that the transition from the darker to the lighter portions of the original image as it will be formed by application of the heat image to the magnetic recording layer will form a raster of composite magnetic particles of different magnetic properties. This is schematically shown in portion I of FIG. 13. Only at the portions of the magnetic recording layer which corresponds to the darkest portions of the original image all four different types of composite grains (each type of composite grains having the same core but a cover layer of different temperature dependency of its permeability) will be magnetized, while at the lighter portions only some of the composite grains or none of them will be magnetized so as to be capable of attracting magnetic ink. The number and size of the different types of composite magnetic grains has to be adjusted to the desired raster dimensions and fineness of the tone value or color intensity gradation desired in the visible copy which is to be formed from the latent magnetic image. Furthermore, the different types of grains should be mixed as evenly as possible and preferably, in order to achieve the desired result, a layer of the magnetic grains should be applied to the support of the recording device or layer which has only the thickness of a single grain. In other words, the magnetic grains should be arranged in one plane adjacent to but not superposed upon each other. Such single grain layer can be easily produced in conventional manner by raking a loose mass of the magnetic composite grains which has been poured onto an adhesive support. It is furthermore possible to admix the composite grains to a conventional printing ink and to print with this mixture a very thin, uniform layer.

It is also possible to produce with the recording layer illustrated in FIG. 6 the halftone points which are shown in portion II of FIG. 13 provided that the various types of grain sheathings or coverings which are of temperature dependent permeability are replaced by coverings of linear temperature dependent permeability or by a uniform carrier layer of linear temperature dependency of its permeability. The magnetization of each of the grains will then continuously increase with

continuous increase in the intensity of the heat image applied to the recording layer. The greater the intensity of the heat image at a given point, the greater will be the lateral extension of its effect until the latent magnetic image portion formed in one grain will grow together with that formed in the adjacent grain.

The shielding effect of the sheathing or covering layer of the composite magnetic grain may be illustrated in the following manner:

10 By inserting into equation (1) (although the same is valid only for a hollow sphere which surrounds a space having a permeability of  $\mu=1$ , which condition is not exactly fulfilled in the case of the composite grain) the actual values for diameters and permeabilities, then a proportionality factor or ratio will be found which indicates the weakening of an external magnetic field which from the outside acts on the composite magnetic grain, and which also indicates the weakening of an internal magnetic field which emanates outwardly from the core portion of the magnetic grain. It may be assumed that this 15 ratio corresponds in both cases exactly to the value 100. This value corresponds in first approximation of the actual value found in the case of composite magnetic grains of the described dimensions and materials. Under these circumstances, for instance, a core portion formed by a permanent magnetic material which has been premagnetized by means of an external magnetic field to a permanent magnetization producing an external field of 1,000 Oerstedts will create a magnetic field which extends outwardly from the core portion through the covering portion of the magnetic grain with a magnetic field strength of 10 Oerstedts and thus the magnetic attraction of the grain with respect to the magnetic particles which contact the recording layer, i.e., the respective grain will have a strength of 10 Oerstedts. The attracting forces 20 which act on such magnetic particles, for instance magnetic ink, depend, apart from the above-discussed magnetic field strength, also on the gradient or inhomogeneity of the magnetic field which, in known manner can be increased, for instance by an appropriate rastering of the field. However, if it is 25 assumed that the residual printing ink is withdrawn after the printing step by an outer magnetic field of comparable inhomogeneity, then this outer magnetic field must possess about twice the strength of the field produced by the printing form or recording layer in order to achieve that the magnetic ink particles which were attracted by the printing form or recording layer will separate therefrom and will with certainty be transferred to the surface of the erasing magnet. In this example, consequently, the magnetic field emanating from the 30 erasing magnet must have a strength of about 20 Oerstedts and thus will exert its effect on the premagnetized core portion of the composite magnetic grain with a strength of 20/100 or 1/5 Oerstedt. In other words, the effect of the erasing magnetic field on the permanently magnetized core portion of the magnetic grain equals one five-thousandth of the magnetic field strength emanating from the core portion of the composite magnetic grain.

FIGS. 14-17 may serve to illustrate a further possibility of applying the heat images of several color separations to a magnetic recording layer so as to form a latent magnetic image or magnetic printing form. According to the presently described embodiment a layer 33 of magnetic material showing a permeability curve corresponding about to curve  $s$  of FIG. 15 is applied to a preferably magnetically inert or neutral carrier layer 22. A magnetic material having a temperature dependency of its permeability corresponding to that shown by broken line  $s$  of FIG. 15 may consist for instance of a cobalt-mixed ferrite of the general formula  $Co_xFe_{3-x}O_4$  or of a mixture of several of the magnetic materials illustrated in FIG. 1. 40 Four permanently magnetizable core particles 34, 36, 38 and 40 which may consist for instance of Bayer S 12 are embedded in magnetic layer 33, and each of the core particles is sheathed or covered with one of the cover layers 35, 37, 39 and 41 which, respectively possess differently temperature dependent 45 permeabilities in accordance with curves  $m35, m37, m39$  and

*m41* of FIG. 15. The approximate activating temperatures of the individual grains as well as the correlation of the individual types of grains to specific colors are indicated in FIGS. 14 and 15.

FIG. 16 shows the magnetization curve of the core material whereby a different range of magnetic field strength is assigned to each different color. Thereby, in conventional manner, the zero point of the permanent magnetization is plotted in the left-hand portion and to the right thereof the strength of the external magnetic field which is required for producing this magnetization along the initial magnetizing curve. One can start from this initial magnetizing curve after an interposed demagnetization in an alternating field of reducing strength, even in the case of recording layers which may be used repeatedly.

If now in addition, each inking arrangement has a threshold value equal to the maximum field strength of the next lower range, then for instance, upon applying the red separation at temperatures of between 70° and 100° C. the "blue" and the "black" grain will be magnetized only to a degree which is insufficient for actuating the corresponding inking arrangements, while, in accordance with FIG. 15, the "yellow" grain is still blocked. The same holds true for the other color ranges. In other words, during application of the individual color separations and simultaneous magnetizing with different field strengths, all grains, the magnetization of which due to the applied external field strength would rise above the threshold value of the correlated inking arrangement, are blocked. The grains which actually belong to a higher color or field strength range thereby automatically become grains of the respectively applied field strength. Since the magnetic grains can replace each other only in the direction from "black" to "yellow" but not in the opposite direction, there will be achieved thereby automatically the effect of the conventional printing technique, namely, that yellow is printed so as to cover the broadest area, while red, blue and black are printed at comparable color intensities with progressively smaller dot areas.

If in the case of a mixed color, for instance, green, the color component which belongs to the higher temperature range, for instance yellow, is applied prior to application of the color component which belongs to the lower temperature range, for instance blue, then the grains which belong to a lower temperature range but to a higher range of magnetic field strength, namely, the "blue" grains will be supplementary magnetized to a higher degree. By applying of the color components in the reverse sequence each grain immediately receives its proper magnetization. The gradation within the color ranges which is required in the case of mixed colors is assured by the characteristics of curve *s* (FIG. 15). In order to obtain in spite of the continuously rising blocking effect the absolute magnetic field strength according to FIG. 16, the strength of the outer magnetic poles 42 to 45 which are schematically shown in FIG. 14, will be correspondingly increased. In case it is undesirable to exchange the grain ranges as described above, then the cores 34, 36, 38 and 40 of the grains as shown in FIG. 17 may be formed of different permanently magnetic or hard magnetic materials, the initial magnetizing curves of which slope at differently steep angles in the vicinity of point zero. For instance, as shown in FIG. 17, a 36 percent cobalt-magnet steel could be used as well as the magnetic alloys which are commercially available under the trade names "Alnico 2" and "Alnico 12." All of the grains belonging to a higher range of magnetic field strengths will then remain not only below the threshold value of the next inking arrangement but also below that of all successively following inking arrangements. For instance, the external magnetic field of between 1,300 and 2,000 Oerstedts which is correlated to the blue range will produce according to the portions of its magnetization loop which are shown in broken lines and indicated as *n'* and *n''*, a permanent magnetization of 1,000 Oerstedts, while the maximum external magnetization of 1,000 Oerstedts which is correlated to the red range will, according to the magnetization loop portion *n'''* cause a permanent magnetization of the "blue" grain of less than 100 Oerstedts.

According to FIG. 18, the individual composite grains of a recording layer which generally corresponds to that of FIG. 15 are surrounded respectively by an additional covering 67 to 70.

During application of the latent magnetic image, these double coverings have an evenly high blocking effect which is compensated by an appropriate increase in the strength of the external magnetic fields 42 to 45 of FIG. 14. Magnetic ink is applied with an inking arrangement according to FIG. 8 according to which each color is offered at a different distance from the recording layer. However, the recording layer is heated in a stepwise manner between the individual applications of colored magnetic ink, for instance in the manner illustrated in FIG. 9.

This will accomplish that before being exposed to the yellow ink supply arrangement both "yellow" coverings will be deblocked or freed while, with respect to the other types of composite grains, only the inner coverings are deblocked. Thus, only the "yellow" grains will be supplied with ink by the yellow inking arrangement. Before reaching the red inking arrangement, additionally the "red" outer covering is deblocked. Since, however, the distance *d*2 of the red inking arrangement is already too great for the "yellow" grains, only the "red" grains are supplied with ink and, in the same manner, successively, the inks of the other colors are supplied. It is also possible to form with this layer containing magnetic grains with two superposed coverings to form copies of several groups of data or information which are at different temperatures, however so that each group is separately printed, or upon appropriate variation of the distance of the various inking arrangements from the recording layer, it is also possible to print several such groups simultaneously.

FIG. 19 shows the connection between the covering of the individual color components and the temperature ranges which are correlated to the different types of composite grains. It is assumed thereby that the layer is first at a starting temperature of 50° C. at which all grains are still blocked. If now heat radiation is applied which without interposition of a filter, or by interposition of a 100 percent permeable original image, would cause, depending only on intensity and length of application of the radiation, a heating of the layer to one of the limiting temperatures indicated at the left hand of FIG. 19, than the actually caused heating of the layer will be reduced in accordance with straight lines E1 to E4, in linear dependency on the percentage density of the original image through which the heat radiation passes. The condition which must be met for forming temperature ranges which do not overlap can now be formulated as the requirement that the respective line E must cross-sect a vertical line passing through the maximum density of the respective color separation at a point which is above the temperature limit of the next lower temperature range.

This is illustrated in FIG. 19 for the densities of the primary color portions which may be found in color transparencies. This representation is applicable for a process wherein the transparency is evaluated at equal exposure times with differently colored light by means of a picture pickup tube whereby the amount of heat produced per unit area in the pickup tube is independent from the color of the light and only proportional to the amount of light which is passed through. However, the representation of FIG. 19 is also suitable when it is intended to form from a colored positive transparency a black and white negative and the latter is then to be penetrated by rays emanating from a source of heat radiation. The individual color separations are then to be exposed in such a manner that each negative in spite of the differences in the maximum color coverage or opaqueness of the positive will obtain at the darkest portions of the positive which correspond to the lightest portions of the negative, a permeability of about 100 percent. For this purpose, the denser positive separations must be exposed for a longer period of time in order to obtain in the negative separations essentially again the initial gradation of maximum densities.

According to FIG. 20, a mixed layer 46 of magnetic materials according to the present invention is placed or applied to the surface of a plate 53 in which electric heating coils 48 to 52 are arranged so that they may be individually connected to a source of electric energy 59 by actuation of switches 54 to 58. Selective actuation of one or the other of the heating coils will permit to heat individual lines or columns of layer 46 to the temperature at which the blocking effect of the highly permeable layer portions is removed. Magnetic ink which is offered, for instance, by means of screen roller 60 will then be attracted only by the deblocked lines or only by certain selected lines of the magnetic printing form.

The electric return conduit 61 includes a bimetal control element 62 or the like which contacts a surface located outside the image area and continuously heated by means of the heating coil 47. Control element 62 will interrupt current supplied to all heating coils as soon as the temperature at the point of comparison exceeds a predetermined temperature.

The heating of selected portion of layer 46 can also be achieved by means of a source 63 of radiant heat by interposition of a stencil 65 which is turnable about shaft 64. Stencil 65 has openings to the portions of the latent magnetic image in layer 46 which are to be reproduced. During the heating by means of heating device 63, stencil 65 rests on support 66 and prior to applying ink, stencil 65 is raised by being pivoted about shaft 64.

It will be understood that each of the elements described above, or two or more together, may also find a useful application in other types of magnetic recording devices differing from the types described above.

While the invention has been illustrated and described as embodied in a magnetic image recording and printing device, it is not intended to be limited to the details shown, since various modifications and structural changes may be made without departing in any way from the spirit of the present invention.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is:

1. In a method of operating a device for storing magnetic recordings, of the type including a raster formed of alternating portions of a hard magnetic material of relatively low permeability and of a material of a relatively high permeability which is temperature dependent within the range of operating temperatures of said recording means, the steps of subjecting said raster at a predetermined temperature in the vicinity of the Curie point of said material of relatively high permeability to a magnetic field; and sweeping said raster at a temperature below said predetermined temperature.

2. In a method of preparing a latent image, the steps of forming a layer including portions of different magnetizable materials in the region of a face of said layer, the magnetic characteristics of each of said materials being adapted to be changed by heating said materials to at least a predetermined different temperature, respectively; and heating said face of said layer selectively to different ones of said predetermined different temperatures in such a manner that each of said different ones of said predetermined different temperatures corresponds to a selected characteristic of an image to be reproduced, so as to change the magnetic characteristics of the materials of those particles which are heated to at least their respective predetermined temperatures, whereby the distribution in said layer of different magnetizable materials the magnetic characteristics of which have been changed corresponds to the distribution of the selected characteristics of said image to be reproduced.

3. In a method of preparing a latent halftone image, the steps of forming a layer including portions of different magnetizable materials in the region of a face of said layer, the magnetic characteristics of each of said materials being adapted to be changed by heating said materials to at least a predetermined different temperature, respectively, each of said different magnetizable materials comprising particles consisting essentially of a core portion of hard magnetic material and a cover layer of soft magnetic material the magnetic permeability of which has a predetermined temperature dependency which is different for each of said different magnetizable materials, respectively; and heating said face of said layer selectively to different ones of said predetermined different temperatures in such a manner that each of said different ones of said predetermined different temperatures corresponds to a selected characteristic of an image to be reproduced, so as to change the magnetic characteristics of the materials of those particles which are heated to at least their respective predetermined temperatures, whereby the distribution in said layer of different magnetizable materials the magnetic characteristics of which have been changed corresponds to the distribution of the selected characteristics of said image to be reproduced.

4. In a method of preparing a latent image of a colored image to be reproduced, the steps of forming a layer including portions of different magnetizable materials in the region of a face of said layer, the magnetic characteristics of each of said materials being adapted to be changed by heating said materials to at least a predetermined different temperature, respectively; and heating said face of said layer selectively to different ones of said predetermined different temperatures in such a manner that each of said different ones of said predetermined different temperatures corresponds to a color separation of said colored image to be reproduced, so as to change the magnetic characteristics of the materials of those particles which are heated to at least their respective predetermined temperatures, whereby the distribution in said layer of different magnetizable materials the magnetic characteristics of which have been changed corresponds to the distribution of the color separations of said colored image to be reproduced.

5. In a method of reproducing a colored image, the steps of forming a layer including portions of different magnetizable materials in the region of a face of said layer, the permeabilities of at least a portion of each of said materials being adapted to be changed by heating said materials to at least a predetermined different temperature, respectively, each of said different magnetizable materials comprising particles consisting essentially of a core portion of hard magnetic material and a cover layer of soft magnetic material the magnetic permeability of which has a predetermined temperature dependency which is different for each of said different magnetizable materials, respectively; heating said face of said layer selectively to different ones of said predetermined different temperatures in such a manner that each of said different ones of said predetermined different temperatures corresponds to a selected color separation of said colored image to be reproduced so as to change the magnetic permeabilities of the materials of those particles which are heated to at least their respective predetermined temperatures, whereby the distribution in said layer of different magnetizable materials to the permeabilities of which have been changed forms a pattern corresponding to the distribution of the color separations of said colored image to be reproduced; and forming from said pattern a reproduction of said colored image by applying thereto magnetic dyestuffs corresponding to said color separations at said respective predetermined temperatures.

6. In a method of reproducing a colored image, the steps of forming a layer including portions of different magnetizable materials in the region of a face of said layer, the permeabilities of at least a portion of each of said materials being adapted to be changed by heating said materials to at least a predetermined different temperature, respectively, each of said different magnetizable materials comprising particles

consisting essentially of a core portion of hard magnetic material and a cover layer of soft magnetic material the magnetic permeability of which has a predetermined temperature dependency which is different for each of said different magnetizable materials, respectively; and heating said face of said layer selectively to different ones of said predetermined different temperatures in such a manner that each of said different ones of said predetermined different temperatures corresponds to a selected color separation of said colored image to be reproduced so as to change the magnetic permeabilities of the materials of those particles which are heated to at least their respective predetermined temperatures, whereby the distribution in said layer of different magnetizable materials the permeabilities of which have been changed forms a pattern of magnetic forces of different strength corresponding to the distribution of the color separations of said colored image to be reproduced.

7. In a method of reproducing a colored image, the steps of forming a layer including portions of different magnetizable materials in the region of a face of said layer, the permeabilities of at least a portion of each of said materials being adapted to be changed by heating said materials to at least a predetermined different temperature, respectively, each of said different magnetizable materials comprising particles consisting essentially of a core portion of hard magnetic material and a cover layer of soft magnetic material the magnetic permeability of which has a predetermined temperature dependency which is different for each of said different magnetizable materials, respectively; heating said face of said layer selectively to different ones of said predetermined different temperatures in such a manner that each of said different ones of said predetermined different temperatures corresponds to a selected color separation of said colored image to be reproduced so as to change the magnetic permeabilities of the materials of those particles which are heated to at least their respective predetermined temperatures, whereby the distribution in said layer of different magnetizable materials the permeabilities of which have been changed forms a pattern of magnetic forces of different strength corresponding to the distribution of the color separations of said colored image to be reproduced; and forming from said pattern a reproduction of said colored image by attracting thereto magnetic dyestuffs corresponding to said color separations at said respective predetermined temperatures from different distances corresponding to the different strengths of said magnetic forces.

8. In a method of reproducing a colored image, the steps of forming a layer including portions of different magnetizable materials in the region of a face of said layer, the permeabilities of at least a portion of each of said materials being adapted to be changed by heating said materials to at least a predetermined different temperature, respectively, each of said different magnetizable materials comprising particles consisting essentially of a core portion of hard magnetic material and a cover layer of soft magnetic material the magnetic permeability of which has a predetermined temperature dependency which is different for each of said different magnetizable materials, respectively; heating said face of said layer selectively to different ones of said predetermined different temperatures in such a manner that each of said different ones of said predetermined different temperatures corresponds to a selected color separation of said colored image to be reproduced so as to change the magnetic permeabilities of the materials of those particles which are heated to at least their respective predetermined temperatures, whereby the distribution in said layer of different magnetizable materials the permeabilities of which have been changed forms a pattern corresponding to the distribution of the color separations of said colored image to be reproduced; and forming from said pattern a reproduction of said colored image by attracting thereto from an equal distance magnetic dyestuffs having different permeabilities corresponding to said color separations at said respective predetermined temperatures.

9. In a method of reproducing a colored image, the steps of forming a layer including portions of different magnetizable materials in the region of a face of said layer, the permeabilities of at least a portion of each of said materials being adapted to be changed by heating said materials to at least a predetermined different temperature, respectively, each of said different magnetizable materials comprising particles consisting essentially of a core portion of hard magnetic material and a cover layer of soft magnetic material the magnetic permeability of which has a predetermined temperature dependency which is different for each of said different magnetizable materials, respectively; heating said face of said layer selectively to different ones of said predetermined different temperatures in such a manner that each of said different ones of said predetermined different temperatures corresponds to a selected information so as to change the magnetic permeabilities of the materials of those particles which are heated to at least their respective predetermined temperatures, whereby the distribution in said layer of different magnetizable materials the permeabilities of which have been changed forms a pattern corresponding to the distribution of the selected informations; and forming from said pattern a colored reproduction of said informations by applying thereto magnetic dyestuffs corresponding to said informations at said respective predetermined temperatures.

10. An inking arrangement for printing an image corresponding to a pattern of different magnetic characteristics formed in a magnetic recording layer, comprising, in combination, ink supply means for supplying magnetic ink of predetermined magnetic force, said ink supply means having a magnetic threshold value below the magnetic force of said magnetic ink; printing roller means adapted to receive ink from said ink supply means and for transferring said ink to a copy sheet, said printing roller means consisting essentially of a ferromagnetic material having a magnetic saturation value which is lower than the magnetic force of said ink by at most the threshold value of said ink supply means, and having prior to reaching the saturation value of said ink a lower total permeability than the latter; and means for adjusting the distance of said printing roller means from said copy sheet.

11. In a device for storing magnetic recordings wherein the temperature dependency of a magnetic characteristic of a magnetic material is utilized for magnetic data recording, recording means for magnetic data recording including a body containing at least two magnetic materials of different temperature dependency of their magnetic permeability, one of said magnetic materials being a subdivided hard magnetic material and the other of said magnetic material being a soft magnetic material the magnetic permeability of which is temperature dependent within the range of operating temperatures of said recording means, said hard magnetic material being embedded in said soft magnetic material.

12. In a device for storing magnetic recordings wherein the difference of the temperature dependency of the permeability of at least two magnetic materials is utilized for magnetic data recording, recording means for magnetic data recording including a coherent layer consisting essentially of a mixture of pulverulent hard magnetic and soft magnetic particles of different permeability within the range of operating temperatures of said recording means.

13. In a device for storing magnetic recordings wherein the difference of the temperature dependency of the permeability of at least two magnetic materials is utilized for magnetic data recording, recording means for magnetic data recording including a coherent layer consisting essentially of a mixture of a mass of pulverulent hard magnetic and a mass of soft magnetic particles of different permeability within the range of operating temperatures of said recording means one of said masses of pulverulent particles exerting a magnetic shielding effect with respect to the other.

14. In a device for storing magnetic recordings wherein the temperature dependency of a magnetic characteristic of a magnetic material is utilized for magnetic data recording,

recording means for magnetic data recording including a thermoplastic synthetic material having a melting point above the operating temperature of said recording means; and at least two pulverulent magnetic materials of different temperature dependency of their magnetic permeability embedded in said synthetic material.

15. In a device for storing magnetic recordings wherein the temperature dependency of a magnetic characteristic of a magnetic material is utilized for magnetic data recording, recording means for magnetic data recording including a thermosetting synthetic material having a decomposition point above the operating temperature of said recording means; and at least two pulverulent magnetic materials of different temperature dependency of their magnetic permeability embedded in said synthetic material.

16. In a device for storing magnetic recordings wherein the temperature dependency of a magnetic characteristic of a magnetic material is utilized for magnetic data recording, recording means for magnetic data recording including a sintered body of at least two magnetic materials of different temperature dependency of their magnetic permeability.

17. In a device for storing magnetic recordings wherein the temperature dependency of a magnetic characteristic of a magnetic material is utilized for magnetic data recording, recording means for magnetic data recording including a body containing at least two magnetic materials of different temperature dependency of their magnetic permeability, one of said magnetic materials being a soft magnetic material the magnetic permeability of which is temperature dependent within the range of the operating temperatures of said recording means, and the other of said magnetic materials being a pulverulent, hard magnetic material, said soft magnetic material forming sintered envelopes surrounding particles of said pulverulent hard magnetic material.

18. In a device for storing magnetic recordings wherein the temperature dependency of a magnetic characteristic of a magnetic material is utilized for magnetic data recording, recording means for magnetic data recording including a body containing at least two magnetic materials of different temperature dependency of their magnetic permeability, one of said magnetic materials being a soft magnetic material the magnetic permeability of which is temperature dependent within the range of the operating temperatures of said recording means, and the other of said magnetic materials being a pulverulent, hard magnetic material, said soft magnetic material forming a coherent sintered body having particles of said pulverulent hard magnetic material embedded therein.

19. In a device for storing magnetic recordings wherein the temperature dependency of the permeability of a magnetic material is utilized for magnetic data recording, recording means for magnetic data recording including a resilient layer of synthetic material; sintered envelopes formed of a soft magnetic material the magnetic permeability of which is temperature dependent within the range of operating temperatures of said recording means embedded in said resilient layer; and particles of a pulverulent hard magnetic material surrounded by said sintered envelopes, respectively.

20. In a device for storing magnetic recordings wherein the temperature dependency of the permeability of a magnetic material is utilized for magnetic data recording, recording means for magnetic data recording including a fibrous layer; sintered envelopes formed of a soft magnetic material the magnetic permeability of which is temperature dependent within the range of operating temperatures of said recording means embedded in said fibrous layer; and particles of a pulverulent hard magnetic material surrounded by said sintered envelopes, respectively.

21. In a device for storing magnetic recordings wherein the temperature dependency of the permeability of a magnetic material is utilized for magnetic data recording, recording means for magnetic data recording including a support; sintered envelopes formed of a soft magnetic material the magnetic permeability of which is temperature dependent within

the range of operating temperatures of said recording means adhesively adhered to said support so as to form thereon a single thickness layer of said envelopes; and particles of a pulverulent hard magnetic material surrounded by said sintered envelopes, respectively.

22. In a device for storing magnetic recordings wherein the temperature dependency of a magnetic characteristic of a magnetic material is utilized for magnetic data recording, recording means for magnetic data recording including a body containing at least two magnetic materials of different temperature dependency of their magnetic permeability, one of said magnetic materials being an elongated body of hard magnetic material and the other of said magnetic material being a layer of soft magnetic material sheathing said elongated body of hard magnetic material, the magnetic permeability of said soft magnetic material being temperature dependent within the range of operating temperatures of said recording means, said hard magnetic material being embedded in said soft magnetic material.

23. In a device for storing magnetic recordings wherein the temperature dependency of a magnetic characteristic of a magnetic material is utilized for magnetic data recording, recording means for magnetic data recording including a body containing at least two magnetic materials of different temperature dependency of their magnetic permeability, one of said magnetic materials being a screen of hard magnetic material and the other of said magnetic material being a layer of soft magnetic material sheathing said screen of hard magnetic material, the magnetic permeability of said soft magnetic material being temperature dependent within the range of operating temperatures of said recording means, said hard magnetic material being embedded in said soft magnetic material.

24. In a device for storing magnetic recordings wherein the temperature dependency of the permeability of magnetic materials is utilized for magnetic data recording, recording means for magnetic data recording including a substantially uniform arrangement of first magnetic bodies consisting essentially of core portions of hard magnetic material and cover layers of a soft magnetic material the magnetic permeability of which has a predetermined temperature dependency within the range of operating temperatures of said recording means, and of second magnetic bodies consisting essentially of core portions of hard magnetic material and cover layers of a soft magnetic material the magnetic permeability of which has a temperature dependency within the range of operating temperatures of said recording means which differs from said predetermined temperature dependency.

25. In a device for storing magnetic recordings wherein the temperature dependency of the permeability of magnetic materials is utilized for magnetic data recording, recording means for magnetic data recording including a substantially uniform arrangement of first magnetic bodies consisting essentially of core portions of hard magnetic material having a predetermined coercive force and cover layers of a soft magnetic material the magnetic permeability of which has a predetermined temperature dependency within the range of operating temperatures of said recording means, and of second magnetic bodies consisting essentially of core portions of hard magnetic material having a coercive force differing from said predetermined coercive force and cover layers of a soft magnetic material the magnetic permeability of which has a temperature dependency within the range of operating temperatures of said recording means which differs from said predetermined temperature dependency.

26. In a device for storing magnetic recordings wherein the temperature dependency of the permeability of magnetic materials is utilized for magnetic data recording, recording means for magnetic data recording including a layer of soft magnetic material having a linear temperature dependency of its magnetic permeability within the range of operating temperatures of said recording means; and, embedded in said layer, a plurality of hard magnetic particles.

27. In a device for storing magnetic recordings wherein the temperature dependency of a magnetic characteristic of a magnetic material is utilized for magnetic data recording, recording means for magnetic data recording including a support; and a raster formed of alternating portions of at least two magnetic materials of different temperature dependency of their magnetic permeability.

28. In a device for storing magnetic recordings wherein the temperature dependency of a magnetic characteristic of a magnetic material is utilized for magnetic data recording, recording means for magnetic data recording including a support; and a raster formed of alternating portions of at least two permanently magnetizable materials having Curie points at

different temperatures within the range of operating temperatures of said recording means.

29. In a device for storing magnetic recordings wherein the temperature dependency of a magnetic characteristic of a magnetic material is utilized for magnetic data recording, recording means for magnetic data recording including a support; and a raster formed of alternating portions of at least two permanently magnetizable materials having different degrees of coercive forces and having Curie points at different temperatures within the range of operating temperatures of said recording means.